

May 15, 1945.

L. S. WILDER

2,376,217

COLOR PHOTOGRAPHY

Filed April 6, 1943

FIG. 1.



FIG. 2.



LOT S. WILDER  
INVENTOR

BY *Newton M. Purvis*  
*R. Frank Smith*  
ATTORNEYS

## UNITED STATES PATENT OFFICE

2,376,217

## COLOR PHOTOGRAPHY

Lot S. Wilder, Rochester, N. Y., assignor to Eastman Kodak Company, Rochester, N. Y., a corporation of New Jersey

Application April 6, 1943, Serial No. 481,988

5 Claims. (Cl. 95—2)

This invention relates to color photography and particularly to a multi-layer photographic material for the preparation of colored pictures.

The incorporation in photographic emulsions of compounds containing active methylene or phenolic hydroxyl groups which couple with the development product of primary aromatic amino photographic developers upon photographic development was described in Fischer U. S. Patent 1,102,028, June 30, 1914. When such couplers are incorporated in multi-layer photographic material which contains emulsion layers sensitive to various regions of the spectrum, the couplers tend to reduce the sensitivity of the emulsion in which they are incorporated. One method which has been proposed for overcoming this objectionable action of the coupler compounds in the emulsions is to incorporate the couplers in a pure gelatin layer situated above or below the corresponding sensitive silver halide layer. This method is described in Schinzel U. S. Patent 2,306,410, December 29, 1942, on page 12. When the couplers are incorporated in a plain gelatin layer in this way, they do not reduce the sensitivity of the emulsion layer and a colored image can be produced. The development product of the developing agent diffuses from the silver halide layer into the adjacent layer containing the coupler. The image produced in this way, however, has poor definition and low maximum density.

It is, therefore, an object of the present invention to provide a multi-layer film containing couplers, which produces maximum dye densities. A further object is to provide a method and means for diminishing the speed loss in photographic coatings containing couplers. A still further object is to provide a method and means for improving the definition of images resulting from coatings containing couplers. Other objects will appear from the following description of my invention.

These objects are accomplished by placing adjacent a normal layer containing silver halide and coupler another layer containing the same or faster silver halide only.

In the accompanying drawing, which forms a part of my invention, the Fig. 1 is a sectional view of a film having sensitive layers not containing coupler coated adjacent layers containing couplers, and Fig. 2 is an enlarged sectional view of a portion of Fig. 1.

In the known process of producing colored photographic images in a multi-layer material as described, for example, in Schinzel U. S. Patent

2,306,410, three silver halide emulsion layers, sensitive respectively to the red, green and blue regions, are coated in succession on a support. The red-sensitive emulsion layer preferably contains a non-diffusing coupler capable of producing a blue-green layers, the green-sensitive emulsion layer contains a non-diffusing coupler capable of producing a magenta dye and the blue-sensitive emulsion layer contains a non-diffusing coupler capable of producing a yellow dye. A yellow filter layer is ordinarily coated between the blue-sensitive emulsion layer and the green-sensitive emulsion layer. The non-diffusing couplers incorporated in the sensitive emulsion layers in this way tend to decrease the sensitivity to light of the emulsion layer, and, therefore, make it necessary to expose the material to light of higher intensity or for a longer time in order to secure the necessary dye density in the image. Schinzel suggested on page 12 of his Patent 2,306,410 that the couplers might be incorporated in gelatin layers situated adjacent the corresponding silver halide layers. For example, the magenta coupler would be incorporated in a gelatin layer adjacent the green-sensitive layer rather than incorporated in the green-sensitive layer itself. This expedient overcomes the objectionable desensitizing of the emulsion layer but has the disadvantage that the definition of the resulting images is poorer and the maximum density lower than when the coupler is incorporated in the sensitive layer itself.

According to my invention, I incorporate the coupler in the sensitive layer itself in the customary manner but provide an extra sensitive layer of the same or faster silver halide without the coupler, adjacent the layer containing the coupler. For example, adjacent the green-sensitive emulsion layer containing the coupler producing the magenta dye I provide a green-sensitive silver halide layer not containing coupler. In the corresponding manner, a red-sensitive silver halide emulsion layer not containing coupler may be provided adjacent the red-sensitive emulsion layer containing the coupler producing the cyan dye. The presence of coupler in an unsensitized layer causes less speed loss than in an optically sensitized layer, hence the need for an extra emulsion layer adjacent the blue-sensitive layer containing the coupler producing the yellow dye is considerably less, but such layer can be employed if desired.

A film of this type is shown in the accompanying drawing in which 10 is a base or support of any suitable material such as cellulose ester, syn-

thetic resin, paper or pigmented cellulose ester. On this support are coated silver halide emulsion layers 11, 12 and 13 sensitive respectively to the red, green and blue spectral regions and containing, respectively, couplers capable of producing blue-green or cyan, magenta, and yellow dyes. Adjacent the red-sensitive emulsion layer 11 there is a gelatino-silver halide emulsion layer 14 sensitive to red light of the same region as layer 11. Adjacent the green-sensitive emulsion layer 12 containing the coupler producing the magenta dye there is a gelatino-silver halide emulsion layer 15 sensitive to green light of the same region as the emulsion layer 12. The emulsion layers 14 and 15 are free of coupler. While they are shown as being adjacent each other, it is also possible to coat the layer 14 nearest the support and to coat the layer 15 on the opposite side of the layer 12. The film also has a yellow filter layer 16 between layers 12 and 13, of any suitable light-absorbing material such as colloidal silver.

When a film of this type is exposed to a colored object or image containing the three primary colors, latent images are produced in each of the five sensitive emulsion layers. If the film is to be developed to a color negative, it is developed immediately after exposure in a color-forming developer such as p-amino-dimethylaniline or diethyl-p-phenylenediamine. This development step produces yellow, magenta and cyan dyes in the respective emulsion layers containing these couplers. In the red-sensitive and green-sensitive emulsion layers 14 and 15 not containing coupler a silver image is produced simultaneously with the color development. This development of silver images in layers 14 and 15 results in the formation of oxidation or development products of the developing agent and these oxidation or development products diffuse somewhat into the adjacent emulsion layers. The development product formed in layer 15 diffuses into layer 12 and the development product formed in layer 14 diffuses into layer 11. Since this diffusion takes place only where the layers 14 and 15 have been exposed and a silver image formed, the development product diffuses into the adjacent layers 11 and 12 where those layers were exposed, as well as to some extent in the toe region which was not exposed. The development product from layers 14 and 15 couples with the couplers or color-forming compounds in layers 11 and 12 and serves to increase the toe dye density produced in those layers. This provides a greater dye density than would be possible without the layers 14 and 15 and, therefore, increases the effective speed of the film, since a greater dye density is deposited for the same exposures than would be possible without these extra layers. At the same time the definition of the dye images is not decreased but is as good as it would be without the extra layers (except in shadows).

The action of the extra layer will be more apparent from a consideration of Fig. 2 of the accompanying drawing which is a sectional view of the two layers 11 and 14 comprising a portion of the film shown in Fig. 1. When these layers are exposed by red light and developed in a color-forming developer, image 17 will be formed in layer 11 and image 18 will be formed in layer 14. These images are indicated in the drawing as triangular figures, the left hand side indicating the portion of minimum density and the right hand side the portion of maximum density. Image 17 will consist of metallic silver and cyan dye because of the coupler incorporated in layer

11. Image 18 will consist only of metallic silver because layer 14 contains no coupler. Because of the reduced sensitivity of layer 11 caused by the presence of the coupler, the image 17 has less toe density than the image 18. This is indicated by the fact that the image 18 extends further to the left (beyond the vertical dotted line in the drawing) than the image 17.

The developer oxidation product from image 18 diffuses somewhat into layer 11. When it enters layer 11 it comes in contact with any coupler in that layer which has not already coupled. Cyan dye is thereby formed wherever the developer oxidation product from layer 14 diffuses into layer 11. This is indicated at 19 as a thin portion of dye near the boundary of layers 11 and 14. Since the dye results from silver formation in layer 14, it will extend further into the toe region than image 17 and when the metallic silver is removed from layers 11 and 14 will serve to increase the toe density of image 17. This is equivalent to increasing the speed of layer 11.

In the production of a sensitive photographic film according to my invention, any known photographic silver halide emulsion of satisfactory speed and definition characteristics may be employed. The green-sensitive and red-sensitive emulsion layers may contain any suitable optical sensitizing dyes and the emulsion layers may contain any of the non-diffusing couplers described in Schinzel U. S. Patent 2,306,410.

The sensitive emulsion layers containing the couplers may also be of the type in which the coupler is incorporated in a water-insoluble, water-permeable material as described in Mannes and Godowsky U. S. Patent 2,304,940, December 15, 1942, and Jelley and Vittum U. S. Patent 2,322,027, granted June 15, 1943. Any of the couplers described in these patents may be employed.

Although I have described my invention by reference to a negative development, it is obvious that it may be used also for reversal development. By proper choice of the silver halide content of the emulsions, the coupler ratio and the thickness and speed relationships of the emulsions used, a wide variety of desirable negative or reversal characteristics can be obtained.

In addition to the use of gelatino-silver halide emulsion layers, I may also employ emulsion layers of silver halide dispersed in suitable cellulose esters or ethers, synthetic resins, albumen or other carriers.

It will be understood that the examples included herein are illustrative only and that my invention is to be taken as limited only by the scope of the appended claims.

I claim:

1. A multi-layer photographic material comprising a support having thereon a plurality of silver halide emulsion layers sensitive to different spectral regions and containing different couplers, and contiguous to at least one of said emulsion layers, a silver halide emulsion layer free of coupler and having a spectral sensitivity substantially the same, and a speed at least as great, as that of the coupler-containing layer to which it is contiguous, said layer free of coupler being in contact with no layer of different spectral sensitivity containing coupler.

2. A multi-layer photographic material comprising a support having thereon three gelatino-silver halide emulsion layers sensitive, respectively, to the blue, green, and red spectral regions

and containing couplers, and contiguous to at least one of said emulsion layers sensitive to a wave-length longer than blue, a gelatino-silver halide emulsion layer free of coupler and having a spectral sensitivity substantially the same, and a speed at least as great, as that of the coupler-containing layer to which it is contiguous, said layer free of coupler being in contact with no layer of different spectral sensitivity containing coupler.

3. A multi-layer photographic material comprising a support having thereon three gelatino-silver halide emulsion layers sensitive, respectively, to the blue, green and red spectral regions and containing couplers contiguous to the green-sensitive emulsion layer but not to the red-sensitive emulsion layer, a gelatino-silver halide emulsion layer sensitive to green light and free of coupler, and contiguous to the red-sensitive emulsion layer but not to the green-sensitive emulsion layer containing the coupler, a gelatino-silver halide emulsion layer sensitive to red light and free of coupler, said layers free of coupler having a speed at least as great as that of the coupler-containing layer to which they are contiguous.

4. The method of increasing the dye densities in a multi-layer silver halide photographic material developed by color-forming development, which comprises in a multi-layer material hav-

ing at least two silver halide layers sensitive to different spectral regions, and containing couplers, incorporating contiguous to at least one of said layers, a layer of silver halide free of coupler and sensitive to the same spectral region and having a speed at least as great as the coupler-containing layer to which it is contiguous, said layer free of coupler being in contact with no layer of different spectral sensitivity containing coupler, exposing and developing said material in a color-forming developer whose development products diffuse to some extent from the non-coupler-containing layer into the coupler-containing layer to strengthen the dye image in said last mentioned layer.

5. A multi-layer photographic material comprising a support having thereon three gelatino-silver halide emulsion layers sensitive, respectively, to the blue, green, and red spectral regions and containing couplers, a yellow filter layer between the blue-sensitive and green-sensitive emulsion layers, and contiguous to the red-sensitive emulsion layer but not to the green-sensitive emulsion layer containing the coupler, a gelatino-silver halide emulsion layer sensitive to red light and free of coupler, said layer free of coupler having a speed at least as great as that of the coupler-containing layer to which it is contiguous.

LOT S. WILDER.